

## UNITED STATES PATENT OFFICE

2,347,143

## DYEING OF TEXTILE FIBERS

Clifford Collier Wilcock, Salford, England, assignor to Courtaulds Limited, London, England, a British company

No Drawing. Application May 30, 1942, Serial No. 445,230. In Great Britain July 17, 1941

## 4 Claims. (Cl. 8—55)

This invention relates to an improvement in the dyeing of textile fibers and in particular to the dyeing of nylon.

I have found that the affinity of nylon for certain dyes, and in particular for direct cotton dyestuffs, which normally are not readily taken up by nylon, can be considerably increased by treating the nylon with water, in the liquid state under pressure, at temperatures above 100° centigrade. The extent of the increase in affinity depends on the temperature employed and appears to attain its maximum at about 150° centigrade at which temperature boiling water exerts a pressure of about 55 lbs. per square inch.

The increase in affinity of nylon by the process according to this invention is not deleteriously affected by the presence of a small proportion of acid or alkali during the heating. Generally speaking, when the process is carried out at a higher temperature the same result can be obtained in a shorter time.

With acetate and acid dyestuffs the effect of the treatment of nylon according to this invention is to give the fiber a better affinity for these dyestuffs at lower temperatures than it previously possessed.

The following examples will serve to illustrate the nature of this invention, which, however, is not limited to these examples.

## Example 1

Nylon yarn is treated in an autoclave with water at 150° centigrade for one hour, the pressure inside the autoclave being about 55 lbs. per square inch. It is then dyed at 90° centigrade for one hour in a bath containing 1 per cent of Chlorazol Blue BS (index No. 406), 5 per cent of 80 per cent acetic acid and 2½ per cent of the material sold under the registered trademark "Calgon T" (the essential basis of which is 40

alkali metaphosphate), 50 parts of the bath being used for each part of nylon yarn. The dye-bath is practically exhausted and a medium heavy blue shade obtained, whereas without such pre-treatment of the nylon yarn, dyeing under similar conditions produces a pale sky blue shade, with an exhaustion of only about 25 per cent.

## Example 2

10 Nylon yarn is treated in an autoclave with water at 130° centigrade at a pressure of 25 lbs. per square inch for one hour, and then dyed as described in the foregoing Example 1. 75 per cent exhaustion of the dyebath is obtained.

## 15 What I claim is:

1. A process for improving the affinity of nylon for direct cotton dyestuffs, acetate dyestuffs and acid dyestuffs, which comprises treating the nylon with water in the liquid state under pressure and at a temperature above 100° centigrade.

2. A process for improving the affinity of nylon for direct cotton dyestuffs, acetate dyestuffs and acid dyestuffs, which comprises treating the nylon with water in the liquid state under a pressure of 55 lbs. per square inch and at a temperature of 150° centigrade.

3. A process for improving the affinity of nylon for direct cotton dyestuffs, acetate dyestuffs and acid dyestuffs, which comprises treating the nylon with water in the liquid state under a pressure of 25 lbs. per square inch and at a temperature of 130° centigrade.

35 4. A process for dyeing nylon which comprises treating the nylon with water in the liquid state under pressure and at a temperature above 100° centigrade and then applying to the treated material a dyestuff selected from the group consisting of direct cotton dyestuffs, acetate dyestuffs and acid dyestuffs.

CLIFFORD COLLIER WILCOCK.